

Sept. 5, 1933.

J. C. PEGRAM

1,925,460

SURFACING MATERIAL AND METHOD OF FORMING SAME

Filed Sept. 13, 1930

Fig. 1



Fig. 2

INVENTOR  
JAMES C. PEGRAM  
BY  
Eduard Schaumberg,  
ATTORNEYS

## UNITED STATES PATENT OFFICE

1,925,460

SURFACING MATERIAL AND METHOD OF  
FORMING SAME

James C. Pegram, Alton, Ill., assignor of one-half to William O. Luly, Alton, Ill.

Application September 13, 1930  
Serial No. 481,606

5 Claims. (Cl. 18—59)

This invention relates to improvements in surfacing material and methods of forming same, and more particularly to a surface covering of a flexible nature adapted particularly for use in covering floors and like surfaces. The example presently to be described consists of one application of the principles of the invention to the construction of a tile flooring.

In the laying of tile floors according to the prevailing practice, a concrete base or foundation, usually of a depth of four to six inches, is regarded as necessary as a foundation structure for the tile surface proper. After the concrete base or slab has been allowed sufficient time in which to set, a cement mud or slush is provided on the top of the slab, into which the tile units are set and leveled. The construction is completed upon permitting the cement mixture last applied to harden and hold the tile in place, after which the tile surface itself may be polished and any paper or foreign substance removed therefrom.

It will appear obvious that the use of concrete on a building floor to a depth of several inches, adds considerably to the loading of the floor; in all cases it is necessary that the floor be especially constructed in the first instance, or afterwards braced, to withstand this dead load. If the tile floor be applied to an old building, it is necessary either to drop the floor level at great expense, a distance equivalent to the total depth of the slabs and tile, say four to six inches, or else to suffer a reduction in available head room as a consequence of the installation of the tile floor.

The present invention is directed to a surfacing material and method of forming same, such that the difficulties above enumerated are obviated, and the time, expense and inconveniences of tile installation are minimized.

In accordance with the preceding remarks, an object of the present invention may be stated as the provision of a tile flooring, resulting from a novel method of manufacture, which will minimize the additional loading incident to the use of a stone-like surfacing material.

A further object is attained by the product and method hereinafter described, in the provision of a stone-like surfacing which may be applied completely to a room of usual size, in a few hours time, instead of requiring from two to three weeks, as under the prevailing practice.

A still further object of the invention is to effect a reduction in material cost of a surfacing product, as well as the labor cost presently incident thereto, to an extent that the total outlay for flooring, for example of the type noted, does not

necessarily exceed one-third of the cost of comparable coverings installed under the heretofore prevailing methods.

Yet another object of the invention is attained in a more durable surface covering of such physical characteristics that cracking and like structural faults prevalent in existing concrete-laid floors, are practically eliminated.

A still further object of the invention is attained in the provision of an improved method of manufacture of a flexible flooring material, which may be distributed and sold in the form of panels, slabs or sheets, and which may be applied in practically all cases without the use of a separate subjacent cushion, foundation or binder.

Yet another object of the invention consists in certain improvements in a method or process of manufacturing a surfacing material which conduces to economy, homogeneity, flexibility, a reasonable degree of elasticity, and complete resistance to any action of water.

Further objects and advantages of the invention will appear as the description proceeds, and from the accompanying drawing illustrating one product, constructed according to the presently preferred method. In the drawing:

Fig. 1 is a fragmentary elevation in perspective of a sheet of flooring material constructed according to the present invention, and Fig. 2 is a vertical section through an inverted sheet of the material in a mold employed in manufacturing same.

Referring now by reference characters to the structure of the example described, the surface of the structure consists of a normally exposed layer of wearing material, shown in the present instance as consisting of units of tile 3. The surfacing material may, however, consist of any suitable wearing product, which may be supplied either in sheet or slab form, or as individual units, as illustrated. Where separate units are employed, they are by preference marginally spaced from each other, substantially uniformly, except as the spaces indicated at 4 are filled with a binding or cementitious material hereinafter described. Disposed immediately below, and closely adhering to the tile units 3, is a layer of a somewhat flexible elastic material, indicated at 5, and consisting by preference of an asphalt cement, the composition of which is hereinafter more fully described in connection with the manufacture of the product. As will best appear from Fig. 2, the layer 5 of cementitious material is caused to extend between the individual tile units 3, as

appears at 4, so that not only the lateral margins of the tile units are completely embraced by the material forming layer 5, but also the under surface of the units 3 are caused adhesively to be gripped or engaged by the cementing material.

Disposed just below, and in close adhesion to the layer of material 5, is a sheet of a plastic substance 6, composed, for example of asphalt paper. The strata 3, 5 and 6 and their relation 10 to each other in the completed structure, clearly appear in Fig. 2, in which the layers are shown in the order described, but with the completed structure in inverted position in a mold 7. This mold consists, by preference, of a relatively 15 shallow pan-like structure of open-top construction and provided with side walls and a bottom which may be cast as a single piece of material. The relation of the mold to the manufacture of the product, and its association with the layers 20 3, 5 and 6 will appear from the ensuing description.

Each of the different layers or strata above referred to will be described in order, preceding a description of the operations incident to the 25 manufacture of the completed product. As is known in the art, the tile units 3 are available to the trade in paper form, i. e., with their finished or wearing surface glued or otherwise adhesively secured to a flexible backing, such as a heavy 30 paper. These papers of tile are usually of substantially rectangular form, and substantially two feet in length and one foot in width. For reasons of convenience, therefore, the product manufactured according to the present invention 35 may assume these proportions and dimensions, and the molds or steel forms, such as 7, are, by preference, made to fit closely the edges or margins of a single paper of tile and hence of a single panel or mat of flooring constructed 40 as herein described. As the tile is furnished to the trade, the units 3 are secured in marginally spaced relation to each other, on the paper backing, thus providing the interstices indicated at 4 and shown in Fig. 2 as occupied by a portion of 45 the material constituting the layer 5. This layer consists, according to present preference, of an asphalt cement as a matrix; obviously other plastic or bituminous products may be used so long as they possess equivalent or comparable 50 physical characteristics. To produce a foundation material capable of withstanding the necessary unit loading, and yet possessing a satisfactory degree of flexibility to conform to the subjacent surface, an aggregate consisting, according 55 to present preference, of clean sand of a size to pass a one hundred mesh screen, together with powdered lime stone of a size passing, for example, a two hundred mesh screen, may be thoroughly mixed with the matrix. A preferred 60 practice is to heat the aggregate materials after mixing, to a temperature of approximately 450° F. Under this treatment the aggregate materials are thoroughly dried. The asphalt is heated to at least 350° F. and while in heated condition, 65 the warm aggregate materials are homogeneously mixed with the asphalt cement, resulting in a compound having the required characteristics.

The asphalt paper constituting the layer 6 appearing in Fig. 2, is available to the trade in roll or sheet form and consists, by preference, in substantial part of a compound closely resembling the material forming the vehicular portion of the layer 5.

The finished product of the present example is 70 formed from the several layers above described

by heating each of the molds 7, in which there has previously been disposed, in inverted position, a paper of the tile 3, with the paper portion disposed against the bottom of the mold, and the normally concealed portion of the tile uppermost in the mold. The tile are heated preferably to a temperature, say between 150° F. and 250° F., and the previously compounded asphalt mixture constituting the layer 5, is poured in place upon the layer of tile until the mold is substantially filled with the compound, existing at this stage as a hot liquid or semi-liquid mass, about level with the top of the form. The layer of asphalt paper 6 previously cut closely to fit the form, is laid upon the layer of compound 5 and pressure uniformly applied to the layer 6, and through this layer in turn to the layers 5 and 3. As a result of this pressure the asphalt compound is leveled, and the effect of the pressure and heat of the mass is closely to bind the layer 6 to the layer 5. At the same time and from the same operation, asphalt compound is forced around and between the individual units 3, thus firmly embedding and adhesively securing these units in the layer 5.

The pressure applied to the several layers of material through the paper 6 may be effected in any of the number of ways known in the art, for example in a hydraulic or screw press, or by rollers subjected to sufficient loading to accomplish the results described.

By preference, in production, a sufficient number of the molds 7 are provided, that each mold may be permitted to retain its contents for at least several hours, to permit the mass to temper 110 or be annealed by a gradual cooling, but in no wise disturbing the completed structure until the mass is uniformly and completely restored to ambient temperature. At this stage the mold is easily separable from the completed product.

The tile mats produced by the method above described may be laid upon an ordinary floor without the use of any material for cementing them in place, since each mat will conform in a very short time, due to its flexibility and elasticity, to any ordinary irregularities in the original floor. The mats or panels may be cemented to each other between their marginal edges as they are laid in place. For cementing and forming the seams between adjacent mats, the same asphalt compound 125 may be used, as described above in connection with the layer 5. Due to the use of the steel forms in molding the individual mats, the mats are uniform and the edges match without difficulty, and so closely that the 130 seam or junction therebetween, is unnoticeable. The present product is easily cut to fit any irregularities and may be laid quickly and neatly by anyone, not requiring skilled labor and the consequent installation expense of the tile constructions heretofore prevailing. In certain very unusual cases where the existing floor is extremely uneven, a sand cushion may be provided over the 135 floor as a leveler.

The product resulting from the method described, combines to a degree not heretofore believed possible, the characteristics of pliability and adaptability to conform with irregularities of old flooring, without adding, to any harmful degree, to the loading of the floor; at the same time a surfacing material formed according to the present method, will withstand a large unit pressure without appreciable surface cavitation. Besides possessing a desirable combination of 140 physical characteristics, the resulting product is 145 150

serviceable, lasting, and at least equal in appearance to the prevailing type of tile floors set in place by the use of concrete.

The drawing necessarily has been confined to an illustration of a single popular type of tile flooring, the units of which are of hexagonal outline, and for this reason each tile mat is characterized by marginal indentations. It will, of course, be understood that not only tile, but any other suitable flooring or surfacing material may be processed to provide a product within the intentment of the present invention, and that for example, where the units 3 are of rectangular conformity, the margins of the mat may be rectilinear instead of serrated, as shown.

The present description has, for the sake of a complete disclosure of a product and method falling within the scope of the present invention, described such product and method in great detail. The description is, of course, to be understood merely in an illustrative and not in a limiting sense, since a great variety of materials may be processed to form a product akin to that specifically described, and yet falling within the scope of the invention as defined by the appended claims.

I claim as my invention:

1. The herein described method of forming a panel of a flexible surfacing material which consists in disposing preformed units of a wearing substance in spaced relation upon a support, filling the space between the wearing units, and covering one surface thereof with a premixed asphalt and mineral mixture, in heating the units and mixture, and in applying pressure to the units of wearing substance and mixture, to effect a structural union thereof.

2. The herein described method of forming a panel of a flexible composition product adapted as a flooring, which consists in inverting pre-shaped, pre-spaced units of a wearing material in a molding form, in heating such material and the form, and while heated, applying a heated bituminous-mineral mixture as a binding and foundation material to and between the units of surfacing material and in pressing said materials into interengaging relation while both materials are heated.

3. The herein described method of forming a bitumastic composition material for use as a flooring or the like, which consists in employing a

mold for the material to be formed, introducing to the mold in spaced relation, heated pre-shaped units of surfacing material, applying to the heated units of surfacing material a heated plastic bitumastic material admixed with more than its own weight of a mineral aggregate, and in applying pressure to said product and material while in the mold.

4. The herein described method of forming panels of a flexible covering for floors and the like, including a hard wearing surface, which consists in providing a metal form, the internal dimensions of which are substantially equal to the size of the panel to be formed, in inverting units of the hard surfacing material in spaced relation in the lowermost portion of the metal form, in heating the units of surfacing material, in superposing thereon in the form, a heated asphaltic mineral compound while in plastic condition, in superposing on the compound a layer of asphaltic material of sheet form, in subjecting the layers of asphaltic material and the units of wearing material to pressure applied to said last named layer, whereby to force the asphaltic compound between and around the surfacing units, and in cooling and tempering the said materials while in the mold, removing the panel after substantial restoration to ambient temperature.

5. The herein described method of forming a flexible composition surfacing material including floor tile, which consists in employing a metal mold conforming substantially to a desired panel size of the flooring material, in heating the mold and while heated, in inverting the tile within the mold, and disposing them in relatively spaced relation therein, in heating the tile before introduction to the mold, in preparing an asphaltic compound composed in greater part of mineral aggregate, and in lesser part of an asphaltic matrix, in heating said compound, and while in plastic form, superposing it on said inverted tile in the mold, so that the compound and tile substantially fill said mold, in cutting a flexible sheet of plastic substance substantially to fit within the mold, in applying the cut sheet to the exposed surface of the asphaltic compound, in subjecting the contents of the mold to pressure uniformly applied thereto, and in permitting the materials to temper within the mold.

JAMES C. PEGRAM. 125

55

130

60

135

65

140

70

145

75

150